

1

3,554,747

## ELECTROSTATIC PRINTING MATERIAL AND METHOD OF ITS PREPARATION

Minoo N. Dastoor, Stow, Ohio, assignor to The Goodyear Tire & Rubber Company, Akron, Ohio, a corporation of Ohio

No Drawing. Filed Oct. 27, 1967, Ser. No. 678,533  
Int. Cl. G03g 5/00

U.S. Cl. 96—1.8

9 Claims

### ABSTRACT OF THE DISCLOSURE

An electrostatic printing material having improved print density and a method of its preparation where the electrostatic printing material comprises an electrically conductive support layer and a second layer, the said second layer comprising a polymeric binder containing a dispersion of a photoconductive material, where the polymeric binder is a polymer comprising from about 50 to about 65 percent by weight units derived from ethyl acrylate, from about 3 to about 10 percent by weight units derived from at least one compound selected from the group consisting of hydroxyethyl methacrylate and hydroxypropyl methacrylate, from about 30 to about 45 percent by weight units derived from styrene and up to about 10 percent by weight units derived from monochlorostyrene.

This invention relates to improved electrostatic printing materials and to a method of their preparation.

In electrostatic printing, an electrostatic printing material is generally prepared by depositing or dispersing a particulate photoconductive material in or on an electrically insulative binder which is itself coated onto an electrically conductive material.

In practicing the direct electrostatic process, the electrostatic printing material is exposed to a suitable corona discharge to produce a uniform electrostatic charge on the surface of the photoconductive material. The charged photoconductive material is then exposed to a light source which has sufficient intensity to discharge the electrostatic charge from the portions of the photoconductive material irradiated by the light. The electrostatic charge is discharged in proportion to the intensity of the light rays striking the material. The image is developed utilizing a liquid or powdered developer to form a visible reproduction of the image.

Electrostatic copying papers producing images having high contrast and high print density are continually sought after. Electrostatic copying papers generally available to the art are sensitive to light rays and require storage in complete darkness for a period of time before being exposed to a corona discharge in order to produce images having high contrast. Such dark-resting periods generally range from a few minutes to an hour or more. These papers require care in handling and adequate storage facilities to prevent undue exposure to light.

Print density is strongly related to the amount of electrostatic charge that can be deposited upon and assumed by the photoconductive material with a given corona discharge. Therefore, a high electrostatic charge on the photoconductive material is generally desired for a high print density and electrically insulative binders which permit the photoconductive material to assume a high electrostatic charge.

It is therefore an object of this invention to provide an electrostatic printing paper having improved print density and dark-resting properties. It is another object to provide a new composition comprising a photoconductive material deposited in an electrically insulative composition. A further object is to provide a method of making

2

the composition and the improved electrostatic printing paper.

In accordance with this invention it has been found unexpectedly that an electrostatic printing material suitable for use in an electrostatic reproduction having improved print density comprises an electrically conductive support layer and a second layer, the said second layer comprising a polymeric binder containing a dispersion of a photoconductive material, where the polymeric binder is a polymer comprising from about 50 to about 65 percent by weight units derived from ethyl acrylate, from about 3 to about 10 percent by weight units derived from at least one compound selected from the group consisting of hydroxyethyl methacrylate and hydroxypropyl methacrylate, from about 30 to about 45 percent by weight units derived from styrene and up to about 10 percent by weight units derived from monochlorostyrene. The polymeric binder preferably has an intrinsic viscosity of about 0.2 to about 0.5 when determined in chloroform as a solvent at 30° C.

The electrostatic printing material can be prepared by a method which comprises coating an electrically conductive support with a solution of the polymeric binder containing the photoconductive material and drying the mixture of the polymeric binder and photoconductive material.

The polymeric binder of this invention is preferably prepared by solution polymerizing a monomer mixture which comprises from about 50 to about 65 percent by weight ethyl acrylate from about 3 to about 10 percent by weight of at least one compound selected from the group consisting of hydroxyethyl methacrylate and hydroxypropyl methacrylate, from about 30 to about 45 percent by weight styrene and up to about 10 percent by weight units derived from monochlorostyrene in the presence of a suitable initiator in a solvent which will yield a polymer having an intrinsic viscosity of from about 0.2 to about 0.5 when the conversion of the monomers to the polymer is at least about 97 percent complete. Although this specification teaches that it is preferred that a solvent is selected which will yield a polymer having an intrinsic viscosity of from about 0.2 to about 0.5 at about at least a 97 percent conversion, this is a characterization of the solvent and it is not required that the monomers be at least 97 percent converted to the polymer. If desired, small amounts of other monomers containing carboxylic groups can be mixed with the monomer mixture to enhance the ability of the polymeric binder to adhere to an electrically conductive substrate. An example of such a material is methacrylic acid when used in amounts of from about 0.1 to about 1.0 part by weight per 100 parts of the polymeric binder.

In the practice of this invention, it has been found that the polymeric binder when prepared by solution polymerizing the monomers has a unique utility for providing electrostatic printing papers having improved print density which do not require a dark-resting time.

Various solvents can be used in the preparation of the solution polymer used for the polymeric binder. Representative of the various solvents are solvent mixtures comprising from about 50 to about 90 percent by weight aromatic hydrocarbons such as xylene, toluene and benzene, and from about 50 to about 10 percent by weight aliphatic hydrocarbons, aliphatic alcohols and alcohol ethers. Representative of various aliphatic hydrocarbons are the pentanes, the hexanes, the heptanes, and the octanes. Representative of the various aliphatic alcohols are ethyl alcohol, propyl alcohol, and butyl alcohols. Representative of alcohol ethers is the mono methyl ether of ethylene glycol.

The solution polymerization reaction can be promoted by various free radical initiators well known to those

skilled in the art for promoting free radical solution polymerizations. Representative examples of the various free radical initiators are benzoyl peroxide, tertiary butyl peroxide, lauroyl peroxide, capryloyl peroxide, and azo-bis-isobutyronitrile.

The amount of free radical initiator employed in the polymerizations may be varied over wide concentrations. Of course, a catalytic amount of the initiator must be employed to cause polymerization of the monomers. The optimum amount of initiator depends on a number of factors such as temperature, reactants used, purity of reactants, reaction times desired and the like. Those skilled in the art will readily determine the optimum catalytic ranges.

A wide range of temperatures can be used for the polymerization such as from about 70° C. to about 120° C. although higher or lower temperatures can be used so long as a polymer having an intrinsic viscosity of from about 0.2 to about 0.5 can be produced when the conversion of the monomer is at least about 97 percent. Usually the time for the polymerization reaction to reach at least about a 97 percent conversion can be various times depending upon the initiator, solvent, and reaction temperature such as from about 5 to about 20 hours. The polymerization reaction can be conducted at atmospheric pressure or, if desired, it can be carried out at sub-atmospheric pressure or super-atmospheric pressure.

In the preparation of the electrostatic printing material of this invention, various photoconductive materials can be used with the polymeric binder to form the photoconductive layer. Representative of such materials are selenium, zinc oxide, cadmium sulfide, cadmium telluride, anthracene, sulfur, and mixtures of these compounds. It is usually preferable to use particulate zinc oxide. General-

at least  $10^{-10}$  ohm $^{-1}$  and usually at least  $10^{-6}$  ohm $^{-1}$  cm. $^{-1}$ .

The following examples illustrate the invention. In the examples, parts and percentages are by weight unless otherwise indicated.

#### EXAMPLES 1-10

A series of electrostatic printing papers were prepared with the polymeric binder of this invention prepared by solution polymerization and are herein identified for the purpose of this specification as Examples 1 through 10.

The polymeric binders for the electrostatic printing papers were prepared by the following method:

A solvent consisting of a mixture of xylene and mono methyl ether of ethylene glycol or butanol was charged to a suitable reactor equipped with a stirrer and reflux condenser. The solvent mixture was heated to cause the solvent mixture to reflux in the reflux condenser. To the reactor was then charged styrene, mono chloro styrene, if used, ethyl acrylate, and hydroxyethyl methacrylate or hydroxypropyl methacrylate in various amounts as shown in Table 1 along with small amounts of free radical reaction initiators such as tertiary butyl peroxide at the higher polymerization temperatures and benzoyl peroxide at the lower polymerization temperatures. Small amounts of methacrylic acid were included to enhance the ability of the polymer to adhere to an electrically conductive substrate. All of the amounts of the reactants in Table 2 are in parts by weight. The monomers were polymerized at the temperature ranges shown in Table 1 for about 10 to 18 hours. The polymeric binders prepared as Examples 1-10 in Table 2 correspond to Examples 1-10 of electrostatic printing papers to be prepared from these polymeric binders.

TABLE I.—PREPARATION OF POLYMERIC BINDER

| Example: | Solvent system      |         |                |                                      |          |                | Initiator |  |
|----------|---------------------|---------|----------------|--------------------------------------|----------|----------------|-----------|--|
|          | Reaction temp., °C. | Xylene  |                | Mono methyl ether of ethylene glycol | Monomers |                |           |  |
|          |                     | Styrene | Ethyl acrylate |                                      | Styrene  | Ethyl acrylate |           |  |
| 1        | 130                 | 50      | 50             | 30                                   | 60       | 110            | 21.0      |  |
| 2        | 75-80               | 80      | 20             | 30                                   | 60       | 110            | 31.5      |  |
| 3        | 75-80               | 80      | 420            | 30                                   | 60       | 110            | 31.5      |  |
| 4        | 75-80               | 90      | 10             | 30                                   | 60       | 110            | 31.5      |  |
| 5        | 75-80               | 90      | 10             | 30                                   | 64       | 16             | 31.5      |  |
| 6        | 120                 | 50      | 50             | 60                                   | 30       | 120            | 21.0      |  |
| 7        | 120                 | 50      | 50             | 30                                   | 70       | 0              | 21.0      |  |
| 8        | 120                 | 50      | 50             | 30                                   | 64       | 66             | 21.0      |  |
| 9        | 120                 | 50      | 50             | 30                                   | 62       | 68             | 21.0      |  |
| 10       | 120                 | 50      | 50             | 30                                   | 60       | 610            | 21.0      |  |

<sup>1</sup> Hydroxyethyl methacrylate containing 2.3 percent by weight of methacrylate acid.

<sup>2</sup> Tertiary butyl peroxide.

<sup>3</sup> Benzoyl peroxide.

<sup>4</sup> Butanol was used instead of the mono methyl ether of ethylene glycol.

<sup>5</sup> 0.1 part methacrylic acid added.

<sup>6</sup> Hydroxypropyl methacrylate containing 2.6 percent by weight of methacrylic acid.

ly the photoconductive materials are used in particle sizes of from about 0.2 to about 2 microns. The amount of the photoconductive material used in the photoconductive layer is generally about 10 to about 1,200 percent by weight based on the solution polymer used in this layer and usually from about 500 to about 700 percent based on the solution polymer is desirable.

In the practice of this invention, the photoconductive material is deposited, and generally it is dispersed in particulate form in a solution of the polymeric binder. It is usually preferred that the insulative film suitable for electrostatic reproduction is prepared by dispersing particles of the photoconductive material in a solution of the said polymeric binder and then allowing the solvent to evaporate from the mixture. Generally, the mixture is coated onto the electrically conductive support following which the solvent is evaporated.

Various electrically conductive materials are generally suitable for use as a base in the electrostatic copying material and are generally known to those skilled in the art. The materials used usually have a specific conductivity of

The solutions of polymeric binders were further diluted with toluene to form coating solutions at about 25° C. according to the following recipe:

| Material:                                                                                              | Parts by weight |
|--------------------------------------------------------------------------------------------------------|-----------------|
| Solution of polymeric binder<br>(50% solids by weight)                                                 | 42              |
| Particulate zinc oxide                                                                                 | 120             |
| Dye (33',55'-tetrabromophenol-sulfone<br>phthalein as a 0.005 gram/milliliter<br>of methanol solution) | 0.006           |
| Toluene                                                                                                | 100             |

The coating solutions were each coated onto electrically conductive papers (obtained as Electrophotographic Base Stock ES-45-AA from the Riegel Paper Corporation) with a number 24 Mayer rod in an amount of about 20 pounds of polymer per ream and dried at about 25° C. to form corresponding Examples 1-10 of electrostatic printing papers each comprising a first layer of particulate zinc oxide as the photoconductive material dispersed with the dye in the dried polymeric binder ad-

hered to the second layer of electrically conductive paper. The electrostatic printing papers were then inserted into a Smith Corona, Marchant No. 33 commercial elec-

polymeric binder and the units derived from styrene and ethyl acrylate in the polymeric binder were adjusted to 37 parts and 52 parts respectively.

TABLE III.—COMPARATIVE EVALUATION OF PREPARED ELECTROSTATIC PRINTING PAPERS

|                                  | SCM paper | Paper (A)<br>(from<br>Example 5) | Paper (B) | Paper (C)    |
|----------------------------------|-----------|----------------------------------|-----------|--------------|
| <b>No dark rest:</b>             |           |                                  |           |              |
| Print density                    | Good      | Excellent                        | Excellent | Excellent    |
| Maximum charge (volts)           | 265       | 485                              | 520       | 515          |
| Charge rate (volts/sec.)         | 4.5       | 7.3                              | 9.1       | 7.5          |
| Dark decay (volts/sec.)          | 0         | 1.0                              | 0         | 3.0          |
| Light decay (volts/sec.)         | 94.6      | 142.6                            | 78.7      | 66.7         |
| Background                       | No        | No                               | Yes       | Yes (slight) |
| <b>After 60 hours dark rest:</b> |           |                                  |           |              |
| Print density                    | Good      | Excellent                        | Excellent | Excellent    |
| Maximum charge (volts)           | 310       | 490                              | 520       | 525          |
| Charge rate (volts/sec.)         | 5.7       | 10.5                             | 8.2       | 9.3          |
| Dark decay (volts/sec.)          | 0         | 0                                | 0         | 3.0          |
| Light decay (volts/sec.)         | 91.2      | 122.6                            | 59.7      | 60.7         |
| Background                       | No        | No                               | Yes       | Yes (slight) |
| Adhesion                         | Fair      | Very good                        | Excellent | Excellent    |
| Solvent resistance (36KB)        | do        | Excellent                        | do        | Do           |
| Zinc oxide tolerance             |           | do                               | do        | Do           |

trostatic copying machine in which they were electrostatically charged by a corona discharge source, exposed to reflected image of printed matter which was exposed to a light source, and developed in the copying machine.

Each of the prepared electrostatic printing papers was evaluated as shown in Table II for print density, adhesion of the polymeric binder to the electrically conductive paper, and whether dark resting is required.

TABLE II.—EVALUATION OF ELECTROSTATIC PRINTING PAPERS

|                 | Print density | Adhesion  | Dark resting required |
|-----------------|---------------|-----------|-----------------------|
| <b>Example:</b> |               |           |                       |
| 1               | Excellent     | Excellent | No.                   |
| 2               | do            | do        | Do.                   |
| 3               | do            | do        | Do.                   |
| 4               | do            | do        | Do.                   |
| 5               | do            | do        | Do.                   |
| 6               | do            | do        | Do.                   |
| 7               | Poor          | Poor      | Yes.                  |
| 8               | Excellent     | Excellent | No.                   |
| 9               | do            | do        | Do.                   |
| 10              | do            | do        | Do.                   |

Comparative results of several prepared electrostatic printing papers and a commercial paper are shown in Table III both with respect to no dark resting of the papers and with respect to a 60 hour dark resting period before exposing the papers to the corona discharge as to print density, maximum charge, charge rate, dark decay, residual charge after 4 seconds, and whether background is present.

The electrostatic printing papers compared in Table III are the paper (A), a commercial electrostatic printing paper obtained as Microstatic Copy Paper Type 450 from the SCM Corporation, the paper (B), prepared according to Example 5, a paper (C), prepared according to Example 5 except that a temperature of about 120° C. was used to prepare the polymeric binder and the units derived from styrene and ethyl acrylate in the binder were adjusted to 42 and 52 parts respectively; and a paper (D), prepared according to the method of Example 5 except that five parts of monochloro styrene were polymerized with the monomers to prepare the

It is known that the photoconductive materials used in this invention generally have an intrinsic sensitivity that lies substantially in the ultra-violet region. Therefore it is the commercial practice to broaden the sensitivity of the photoconductive materials over a wider spectrum by mixing small amounts of various dyes which are generally known as dye sensitizers with the photoconductive materials. The dye sensitizers cause the photoconductive materials to be more sensitive, for example, to visible light. Many dye sensitizers can be used and are well known to those skilled in the electrostatic printing art. They are used in the practice of this invention to facilitate the use of the invention over a broader range of light spectrum. When dye sensitizers are used they are normally mixed with the photoconductive material in an amount of 0.1 to about 5 percent and preferably from about 0.1 to about 3 percent. Representative of the many suitable dye sensitizers are, for example, sensitizers of the phenolsulphonephthalein group, phthalain dyes, triphenylmethane dyes and cyanide dyes.

While certain representative embodiments and details have been shown for the purpose of illustrating the invention, it will be apparent to those skilled in this art that various changes and modifications may be made therein without departing from the spirit or scope of the invention.

What is claimed is:

1. An electrostatic printing material not requiring dark resting which comprises an electrically conductive support layer and a second layer, the said second layer comprising a polymeric binder containing a dispersion of a photoconductive material selected from the group consisting of selenium, zinc oxide, cadmium sulfide, cadmium telluride, anthracene and sulfur, where the said polymeric binder is a polymer having an intrinsic viscosity in chloroform at 30° C. of from about 0.2 to about 0.5 prepared by solution polymerization comprising from about 50 to about 65 percent by weight units derived from ethyl acrylate, from about 3 to about 10 percent by weight units derived from at least one compound selected from the group consisting of hydroxyethyl methacrylate and hydroxypropyl methacrylate, from about 30 to about 45 percent by weight units derived from styrene and up to about 10 percent by weight units derived from monochlorostyrene.

2. An electrostatic printing material according to claim 1 where the polymeric binder contains a dispersion of a photoconductive material and a dye sensitizer and the electrically conductive support layer has a specific conductivity of at least about  $10^{-10} \text{ ohm}^{-1}$ .

3. The electrostatic printing material according to claim 2 where the solution polymerization is conducted at a tem-

perature of from about 70° C. to about 120° C., with the solvent mixture comprising from about 50 to about 90 weight percent aromatic hydrocarbons and correspondingly from about 50 to about 10 weight percent aliphatic hydrocarbons and where the conversion of the monomers is at least about 97 percent.

4. An electrostatic printing material according to claim 1 where the photoconductive material is a particulate zinc oxide.

5. A method of preparing the electrostatic printing material of claim 1 which comprises coating an electrically conductive support with a solution of a polymeric binder containing a photoconductive material and drying the mixture of the polymeric binder and photoconductive material where the said polymeric binder is prepared by solution polymerizing a mixture of monomers which comprises from about 50 to about 65 percent by weight ethyl acrylate, from about 3 to about 10 percent by weight of at least one compound selected from the group consisting of hydroxyethyl methacrylate and hydroxypropyl methacrylate, from about 30 to about 45 percent by weight styrene and up to about 10 percent by weight units derived from monochlorostyrene.

6. A method according to claim 5 where the said mixture of monomers is polymerized in the presence of a free radical initiator and a solvent which will yield a polymer having an intrinsic viscosity of from about 0.2 to about 0.5 when the conversion of the mixture of monomers to the polymer is at least about 97 percent complete.

7. A method according to claim 6 where the solvent is a mixture comprising from about 50 to about 90 percent by weight aromatic hydrocarbons and from about

50 to about 10 percent by weight of compounds selected from the group consisting of aliphatic hydrocarbons, aliphatic alcohols and alcohol ethers.

8. A method according to claim 7 where the aromatic hydrocarbons are selected from the group consisting of xylene, benzene, and toluene, the aliphatic hydrocarbons are selected from the group consisting of the pentanes, the hexanes, the heptanes, and the octanes, the aliphatic alcohols are selected from the group consisting of ethyl alcohol, propyl alcohol, and butyl alcohol, and the alcohol ether is a mono methyl ether of ethylene glycol.

9. A method according to claim 6 where the solution of the polymeric binder contains a dispersion of a photoconductive material and a dye sensitizer and where the photoconductive material is selected from at least one of the group consisting of selenium, zinc oxide, cadmium sulfide, cadmium telluride, anthracene and sulfur.

#### References Cited

##### UNITED STATES PATENTS

|           |        |             |       |         |
|-----------|--------|-------------|-------|---------|
| 3,245,833 | 4/1966 | Trevoy      | ----- | 117—201 |
| 3,251,687 | 5/1966 | Fohl et al. | ----- | 96—1    |
| 3,447,957 | 6/1969 | Behringer   | ----- | 117—201 |
| 3,454,415 | 7/1969 | Bonjour     | ----- | 117—34  |

GEORGE F. LESMES, Primary Examiner

M. B. WITTENBERG, Assistant Examiner

U.S. Cl. X.R.

96—1, 1.5; 117—201; 260—80.75